

May 29, 1923.

1,457,285

J. K. SHAW

WALL BOARD MADE FROM BAGASSE AND ANALOGOUS FIBERS

Filed Oct. 23, 1920

Fig. 1.



Fig. 2.



Fig. 3.



Fig. 4.

\_\_\_\_\_  
Inventor  
John K. Shaw, by  
T. G. Witherspoon  
Attorney

Patented May 29, 1923.

## UNITED STATES PATENT OFFICE.

JOHN K. SHAW, OF MINNEAPOLIS, MINNESOTA.

WALL BOARD MADE FROM BAGASSE AND ANALOGOUS FIBERS.

Application filed October 28, 1920. Serial No. 419,045.

*To all whom it may concern:*

Be it known that I, JOHN K. SHAW, a citizen of the United States, residing at Minneapolis, in the county of Hennepin and State of Minnesota, have invented certain new and useful Improvements in Wall Boards Made from Bagasse and Analogous Fibers; and I do hereby declare the following to be a full, clear, and exact description 10 of the invention, such as will enable others skilled in the art to which it appertains to make and use the same.

This invention relates to fiber wall boards made from bagasse and analogous fibers and has for its object to provide a product of this nature which will be more efficient in use and less expensive to produce than those heretofore proposed.

With these and other objects in view the invention consists in the novel details of construction constituting the board, all as will be more fully hereinafter disclosed and particularly pointed out in the claims.

Referring to the accompanying drawings 25 forming a part of this specification in which like numerals designate like parts in all the views:

Figure 1 is a diagrammatic sectional view of a machine suitable for making boards 30 from bagasse and analogous fibers in accordance with this invention;

Figure 2 is a diagrammatic side elevational view of a board made in accordance with this invention;

Figure 3 is an exaggerated diagrammatic 35 sectional view illustrating the construction of a bagasse bundle of fibers with its outer casing partially removed; and

Figure 4 is likewise an exaggerated diagrammatic view illustrating a bundle of 40 bagasse fibers after the outer casing has been removed.

In order that the precise invention may be the more clearly understood the process of 45 preparing fibers and the manner of interweaving or entangling the same will be disclosed, and then the differences between this board and the prior boards will be pointed out.

As regards the process of preparing bagasse and analogous fibers for making this 50 particular wall board, it is well known that not only bagasse fibers but a large number of other fibers have been heretofore treated 55 by boiling with caustic soda and other solu-

tions for the purpose of making paper therefrom, but in so far as I am aware, all of such prior treatments have been more or less drastic in that in order to make paper, it is necessary to use comparatively large 60 quantities of alkali in the solution, and it is necessary that the boiling be prolonged beyond the point at which the particular fiber product useful for making this wall board 65 can be produced.

In addition to this, when using bagasse fibers the prior processes have invariably either mechanically denuded said fibers of their pith before the treatment with the alkali solution, or else the chemical treatment has been carried out for such a length 70 of time as to dissolve said pith. The result, in either case, has been that the prior finished fibers, unlike those produced for making this board, have been substantially 75 smooth and devoid of their natural pith, while more or less of the cellulosic content of the fibers themselves has been dissolved out and lost.

In making fibers to be used in the wall 80 board forming the basis of this invention, on the other hand, although I may employ any suitable chemical to cook the same, yet I prefer a solution of caustic soda. I may use either a strong solution for a very short 85 time, or I may use a weak solution for a longer time, but in all cases the total time of cooking is very much shorter than has heretofore been customary in treating bagasse and analogous fibers. That is to say, 90 I may, for example, take a weight of caustic soda which may be equal only to say about 5% of the bone dry weight of the bagasse, but, of course, said weight of caustic soda would vary from, say, 2% to 10%, or higher, 95 of the bone dry weight of the bagasse. I then make a solution of this said caustic soda and water and heat the bagasse fibers in this solution, to, say, from 1 to 4 hours at atmospheric pressure, and at a temperature of from, say, 150° F. to 212° F., depending 100 upon the physical nature of the particular fibers being treated.

In all cases, whether using a weak or a strong solution in the cooking operation, I 105 am careful to only treat the fibers sufficiently to loosen up the outer encrusting casing of said fibers so that when the latter are passed through a beating engine and a sieving apparatus, this said encrusting casing may be 110

readily and mechanically separated from the fibers themselves.

In other words, referring more especially to Figure 3, an important feature of this treatment resides in the fact that the cooking action is stopped as soon as the outer casing 1 is loosened up from the bundle of fibers 2, and before the accompanying pith is dissolved out, and also before any valuable cellulosic content of the fibers has been lost.

By thus partially cooking the bagasse and analogous fibers I find that I can secure from, say, 65% to 80% of the bone dry weight of the original material, which is a yield almost double that of any previous process of treatment with which I am acquainted. It should be said, however, that this relatively large yield of material is due partially, at least, to the fact that substantially all of the pith originally associated with the fibers is found to remain therewith and to form valuable felting protuberances, as will appear more fully hereinafter.

Not only does the partial cooking of the fibers produce the important results just set forth, but in addition to this, I find that the strength of the original fibers 2 is not impaired in the least, which is in marked contrast to the effect produced by the prior processes, which so drastically cook the same that the original strength of the fibers is very materially lessened.

It is further found in this said partial cooking operation that the alkali or other chemical employed forms valuable water soluble compounds with the casing material 1, and its associated constituents. These said compounds may be re-precipitated, later, upon the fibres, as by adding aluminium sulphate to the solution, so that the fibers in the finished board may be firmly bound together as well as waterproofed.

The fibers having been partially cooked, as above disclosed, the individual bundles of fibers 2 are passed into any suitable beating apparatus and through any suitable screening apparatus, not shown, whereupon the casing material 1 is removed. After this mechanical treatment the character of an individual bundle of fibers 2, will be best understood by reference to Figure 4. That is to say, certain individual fibers lettered 3 in Figure 3, will be found to be broken and their ends will form hook like projections also lettered 3 in Figure 4. Also, the pith having been dissolved as above stated, will be found to be clinging to the bundles of fibers 2 and will form the protuberances or projections 4 illustrated in Figure 4.

In other words, the fibers 2 thus produced will be found unusually strong and flexible and to be very rough on their exterior as

is indicated in Figure 4, with the result that they are capable of interlocking or entangling with each other, or felting together, in the true sense of the word, just as do wool fibers, a result not heretofore attained in vegetable fiber boards, as far as I am aware. Said fibers 2 illustrated in Figure 4, of course, are broken up by the beating engine into much shorter lengths than said figure indicates, the particular length depending upon the mechanical treatment thereof, and they are mixed with water and fed through a pipe 5, Figure 1, to the tank 6, so that a mixture of fibers and water 7 passes up and down between the baffles 8, and thus become thoroughly mixed together.

The water is preferably maintained at a head 9 above the belt or traveling foraminous surface 10, so that the mixture of fibers and water will pass in the direction of the arrows to said traveling foraminous surface 10, whereupon the water will pass through and escape by the passage 11, while the fibers themselves will strike said belt 90 in a direction more or less transversely to its direction of travel, and will be carried along with said belt to the point 12, as will be readily understood.

Other portions of said water will escape through the rotating foraminous surface 13 of the drum 14, other portions of said fibers will likewise strike said surface 13 in a direction more or less perpendicular to its direction of travel, and the latter will likewise be carried toward the point 12.

In the meantime, the third portion of the fibers will be carried between the two sets of fibers thus formed, on the surfaces 10 and 13, and will be likewise carried to the converging point 12, so that all the fibers will be entangled or felted with each other. But individual fibers 2, having the interlocking projections 3 and 4, as illustrated in Figure 4, will by the actions just disclosed be so positively interlocked, and strongly interwoven, or felted together, that the homogeneity and tenacity of the resulting board will be much greater than in prior boards.

In addition to this, the individual strength of said fibers due to the treatment above disclosed, being so much greater than that of wood or other fibers which have been heretofore employed in boards of this same general character, this board is very much stronger and it wears very much better in use than any other analogous product with which I am familiar. Of course, it is understood that after the above three classes of intertwined fibers have been brought to the point 12 they suffer a slight compression between the said surfaces 10 and 13, and also as they pass between the drum 14 and the roll 16, so that the board 17 emerges from the machine as illustrated in Figure 1.

The amount of compression that is imparted to the board 17 will depend upon the use to which it is to be put. If the finished product is to be used as a wall covering, and as a heat insulator, the pressure imparted is not very great; because in that case the board should contain a comparatively large quantity of air in its body portion, and in such cases, I prefer to give it only such a pressure as will cause it to have a specific gravity comparable to that of cork, for I then find that its heat insulating powers are also about as great as cork.

In order to enhance the heat insulating properties of the board, I feed to the mixture 7 coarse fibers 20 as well as fine fibers 21. The former provide relatively large air cells, after the board is compressed, and the latter divide up said cells, add strength and act as a filling material. In other cases, when I wish to add density to the board, without materially impairing its heat insulating qualities, I add wood, flax, or other fibers 22 of various sizes. Such latter boards may have, say, from 10% to 90% bagasse fibers, and from 90% to 10% of other fibers admixed therewith.

On the other hand, if the board is required to have greater strength, then I compress it to such a degree as will cause it to have the desired tenacity and density. It may then be in some cases, compressed to such a degree as to be hard and firm like lumber, when it will be found stronger than many grades of lumber, and to be capable of being sawed, nailed, and hammered, precisely as lumber. Especially does such a board make a valuable substitute for high grades of lumber to be used in trunks, suit cases, furniture, etc.

A lesser compression, however, will make the board softer and more pliable and thus enable it to be used in place of other softer kinds of lumber.

Actual tests have shown boards compressed to 400 pounds to the square inch when made in accordance with this invention, to possess a tensile strength exceeding 12,000 pounds, while similar boards made of flax, wood and other fibers according to the prior processes, only showed a tensile strength of about 1,100 pounds, or less than one tenth the strength of this board.

In my copending application Serial No. 368,995, filed March 26, 1920, and entitled Fiber boards of felted interlaced fibers, I have disclosed and claimed a board similar to this invention, but in that case the board is composed of distinct layers of fibers, differing distinctly from this board. In this board, on the other hand, ordinary felting machines may be employed and the layers of material differing in kind from the body of the board are not produced.

It is obvious that those skilled in the art

may vary the details of construction without departing from the spirit of the invention, and therefore, I do not wish to be limited to the above disclosure except as may be required by the claims.

What I claim is:

1. The herein described fiber board composed of bundles of fibers interlaced with each other, and more than ten per cent of said fiber bundles carrying natural pith like protuberances and hook like projections serving as entangling agents between the fibers, substantially as described.

2. The herein described fiber board composed of fibers interlaced with each other, and more than thirty per cent of said fibers carrying natural pith like heat insulating protuberances and hook like projections serving as entangling agents between the fibers, substantially as described.

3. The herein described fiber board composed of pith carrying bundles of fibers interlaced with each other, said fibers carrying their pith in the form of protuberances attached to the individual fiber bundles and having hook like projections which offer resistance when one fiber bundle tends to slip over another fiber bundle, substantially as described.

4. The herein described fiber board composed of pith carrying bagasse fibers interlaced with each other, said fibers carrying their pith in the form of protuberances attached to the individual fibers which offer resistance when one fiber tends to slip over another fiber, substantially as described.

5. The herein described heat insulating fiber board composed of bagasse fibers of different sizes carrying their natural pith and interlaced with each other, substantially as described.

6. The herein described fiber board composed of bagasse fibers interlaced with each other and carrying their natural pith, said fibers being highly compressed together to form a board of great tensile and breaking strength for use as a substitute for lumber or leather in the manufacture of furniture, baggage and other articles, substantially as described.

7. The herein described fiber board composed of pith carrying bagasse fibers interlaced with each other and admixed with other different kinds of fibers, substantially as described.

8. The herein described fiber board composed of pith carrying bagasse like fibers interlaced with each other and admixed with more than 10% of wood fibers, substantially as described.

9. The herein described fiber board composed of pith carrying fibers in the form of bundles of fibers having hook like projections, said bundles being interlaced with each other and bound together by a com-

pound dissolved from said fibers when in their natural condition, substantially as described.

10. The herein described fiber board composed of pith carrying bagasse fibers interlaced with each other; said fibers being in the form of bundles of different sizes; and

said bundles being bound together by a compound dissolved from said fibers when in their natural state, substantially as de- 10 scribed.

In testimony whereof I affix my signature.

JOHN K. SHAW.